

1

2,934,047

## OPERATION OF INTERNAL COMBUSTION ENGINES OF THE COMPRESSION IGNITION TYPE

Robert D. Young, Hammond, Ind., assignor to Sinclair Refining Company, New York, N.Y., a corporation of Maine

No Drawing. Application August 13, 1951  
Serial No. 241,705

4 Claims. (Cl. 123—1)

My invention relates to a starting fluid for use in compression ignition engines which is particularly valuable in cold weather for low temperature starting.

It is well known that compression ignition engines employing regular diesel fuels are difficult to start under conditions of low ambient temperature particularly at temperatures below about 32° F. In starting a cold engine, the temperature within the cylinder must be sufficiently high to ignite the regular fuel. Such temperatures are developed only after sufficient work has been done in compression of the charges within the working cylinder to bring the parts of the engine in direct heat exchange relation with the contents of the working cylinder, as well as the charge undergoing compression, to a relatively high temperature. Thus, at low ambient temperatures it is often difficult, if not impossible, to attain such required temperatures without special equipment and starting methods.

With the widespread use of diesel engines, particularly in mobile auto-powered equipment in the transportation and construction fields, cold weather starting difficulties for such engines often involve serious economic loss above the mere delay in use of the automotive equipment, hence considerable time and attention have been given to the problem of obtaining reliable and inexpensive cold weather starting methods. Such methods employ winterizing techniques and mechanical starting aids, for example, combustion type air induction heaters, external heaters for engine jacket coolants, jacketed crankcases and the like.

One such method for starting of compression ignition engines contemplates the use of an auxiliary fuel, a starting fluid, in combination with the regular, primary fuel. The auxiliary fluid is aspirated with the engine air intake during starting until combustion of the regular injected fuel is continuous.

I have discovered that volatile organic nitrates, particularly alkyl nitrates, e.g. amyl nitrate, possess specially desirable properties which render them useful aids in cold weather starting of diesels. I have also discovered that blends of amyl nitrate and diethyl ether possess additional extremely useful properties highly desirable in diesel starter fluids. My invention provides a starting fluid containing about 5-95% by volume of diethyl ether and about 95-5% by volume of amyl nitrate. I prefer compositions within the approximate range of about 5-50% by volume of diethyl ether and about 95-50% by volume of amyl nitrate. I particularly prefer a composition of about 20% diethyl ether and 80% amyl nitrate (parts by volume).

In evaluating the relative effectiveness of a given diesel fuel one of the primary criteria of low temperature starting is the minimum compression ratio required for starting the engine. Thus, using the same engine and the same jacket and air temperatures, different fuels may be conveniently evaluated in the laboratory for their cold weather starting performance by comparison of this

2

critical compression ratio. The test is referred to as CCRD test (critical compression ratio differential). The CCRD data have been previously correlated with actual cold weather experiments and have been demonstrated to provide accurate relative prediction of cold weather starting. Such data are to be preferred to actual cold tests as they are more economical and more readily obtained. Where herein referred to, the CCRD data were derived under the following conditions using a CFR

10 Waukesha diesel test unit (1937):

Jacket temperature ----- 30° F.  
Air intake temperature ----- 38° F.  
Primary fuel injection rate ----- 13 cc. per minute.

15 To evaluate the starting characteristics and effectiveness of secondary fuel aspirated with the air intake, the further test conditions were employed.

20 Primary fuel used ----- 50 cetane number Mid Continent diesel fuel.

Quantity secondary fuel aspirated per trial ----- 5 cc.

25 The engine was constantly motored at 900 r.p.m. under equilibrium conditions. The initial compression ratio for the engine was set below the point at which ignition of the primary fuel occurred for an injection duration of 10 seconds. From this point the compression ratio was 30 gradually raised at 10 second intervals until the critical compression ratio of the primary fuel was reached, as evidenced by continuous combustion of the fuel. When this value was determined by three separate determinations, the compression ratio was again substantially lowered and the critical ratio of the primary fuel plus aspirated secondary fuel was determined in like manner. 35 The difference between the two values represents the critical compression ratio difference (CCRD) of the secondary fuel.

40 Under these test conditions the CCRD data were determined using as starting fluids diethyl ether, a proven and well known auxiliary starting fluid, amyl nitrate, and a blend of amyl nitrate and diethyl ether in a 4:1 volume ratio. The following table illustrates the results:

|                                           | Amyl nitrate | 80% (vol.)<br>Amyl nitrate,<br>20% (vol.)<br>Diethyl Ether | Diethyl Ether |
|-------------------------------------------|--------------|------------------------------------------------------------|---------------|
| 50                                        |              |                                                            |               |
| CCRD value-----                           | 3.75         | 5.50                                                       | 4.40          |
| Cetane number-----                        | 275          | 100                                                        | 100           |
| Boiling range, ° F.-----                  | 305          | 100-305                                                    | 94            |
| Pour Point, ° F.-----                     | -139         | -146                                                       | -176          |
| 55 Vapor Press. at 100° F., p.s.i.a.----- | 0.16         | 5.7                                                        | 16.7          |

As the above table shows, amyl nitrate is almost as effective a secondary fuel as diethyl ether, having a 60 CCRD value close to that for diethyl ether. However, amyl nitrate is not as useful in extremely cold weather since it has low volatility. The blend of amyl nitrate and diethyl ether illustrated, however, surmounts these difficulties, having the requisite low pour point characteristics and volatility for atomization with the air intake even under severely low temperatures. Moreover, as is 65 illustrated by the above data, the blend exhibits better starting characteristics, as measured by the CCRD data, than are exhibited by either amyl nitrate or diethyl ether alone, which is indeed a surprising result as diethyl ether 70 is one of the most effective of such fluids previously known.

Additional tests were made to determine the overall ranges of proportions exhibiting these surprising results. The following table is illustrative: (all parts by volume)

| Amyl<br>Nitrate,<br>vol.<br>Percent | Diethyl<br>Ether,<br>vol.<br>Percent | CCRD<br>Value |
|-------------------------------------|--------------------------------------|---------------|
| 100                                 | 0                                    | 3.75          |
| 90                                  | 10                                   | 5.25          |
| 80                                  | 20                                   | 5.50          |
| 70                                  | 30                                   | 5.30          |
| 60                                  | 40                                   | 5.30          |
| 50                                  | 50                                   | 5.25          |
| 40                                  | 60                                   | 5.25          |
| 20                                  | 80                                   | 5.25          |
| 0                                   | 100                                  | 4.40          |

Thus, the improvement exists over an extended range within the approximate limits of about 5%–95% by volume of diethyl ether and about 95%–5% by volume of amyl nitrate. Moreover, within the range of about 5%–50% by volume of diethyl ether and about 95%–50% by volume of amyl nitrate, the blends are not subject to the usual disadvantages of diethyl ether. Burning is smooth and detonation difficulties are overcome. In all blends the volatilities were sufficient for aspiration with the air intake under severely cold weather conditions, yet such volatilities were insufficient to amount to a hazardous problem in warm weather and consequently the blended fluids may be conveniently stored and handled.

The manner in which starting fluids are best used is known to the art. For details and different suggested methods of aspiration I make reference here to my co-pending application Serial No. 84,733, filed March 31, 1949, for Diesel Starting Fluid, now U.S. Letters Patent No. 2,575,543, issued November 20, 1951.

I claim:

1. In the operation of internal combustion engines of the compression ignition type, the improvement which

comprises burning a primary fuel while introducing with the air supply an auxiliary fuel consisting essentially of about 5% to 95% by volume of diethyl ether and about 95% to 5% by volume of amyl nitrate.

5. 2. In the operation of internal combustion engines of the compression ignition type, the improvement which comprises burning a primary fuel while introducing with the air supply an auxiliary fuel consisting essentially of about 5% to 50% by volume of diethyl ether and about 95% to 50% by volume of amyl nitrate.

10. 3. In the operation of internal combustion engines of the compression ignition type, the improvement which comprises burning a primary fuel while introducing with the air supply an auxiliary fuel consisting essentially of about 20% by volume of diethyl ether and about 80% by volume of amyl nitrate.

15. 4. In the operation of internal combustion engines of the compression ignition type, the improvement which comprises burning a primary fuel while introducing with the air supply an auxiliary fuel consisting essentially of 95% to 50% by volume of diethyl ether and about 5% to 50% by volume of amyl nitrate.

#### References Cited in the file of this patent

##### UNITED STATES PATENTS

|           |             |               |
|-----------|-------------|---------------|
| 2,143,870 | Ellis       | Jan. 17, 1939 |
| 2,158,050 | Bereslavsky | May 16, 1939  |
| 2,243,471 | Olin        | May 27, 1941  |
| 2,516,787 | Moody       | July 25, 1950 |
| 2,575,543 | Young       | Nov. 20, 1951 |

##### FOREIGN PATENTS

|         |               |               |
|---------|---------------|---------------|
| 294,129 | Great Britain | July 16, 1928 |
| 600,367 | Great Britain | Apr. 7, 1948  |

##### OTHER REFERENCES

"Lang's Handbook of Chemistry," 4th ed. 1941 p. 286, Handbook Publishers, Inc., Sandusky, Ohio.